

June 2, 1953

S. A. HERRES

2,640,860

APPARATUS FOR MELTING TITANIUM TO FORM INGOTS

Filed Oct. 21, 1949

6 Sheets-Sheet 1



Schuyler A. Herres  
BY Thomas G. Miller  
FOR Green, McCallister & Miller  
HIS ATTORNEYS

June 2, 1953

S. A. HERRES

2,640,860

## APPARATUS FOR MELTING TITANIUM TO FORM INGOTS

Filed Oct. 21, 1949

6 Sheets-Sheet 2



June 2, 1953

S. A. HERRES

2,640,860

APPARATUS FOR MELTING TITANIUM TO FORM INGOTS

Filed Oct. 21, 1949

6 Sheets-Sheet 3



Fig. 7



Fig. 9



Fig. 8

Fig. 7A



Fig. 10



Fig. 11

INVENTOR.

Schuyler A. Herres

BY Thomas G. Miller

FOR Green, McCallister & Miller

HIS ATTORNEYS

June 2, 1953

S. A. HERRES

**2,640,860**

## APPARATUS FOR MELTING TITANIUM TO FORM INGOTS

Filed Oct. 21, 1949

6 Sheets-Sheet 4



Fig. 12

INVENTOR.

*Schuyler A. Herres*

BY *Thomas G. Miller*

Thomas J. Miller  
FOR Green, McCallister & Miller

**HIS ATTORNEYS**

June 2, 1953

S. A. HERRES

2,640,860

## APPARATUS FOR MELTING TITANIUM TO FORM INGOTS

Filed Oct. 21, 1949

6 Sheets-Sheet 5



1 INVENTOR,  
Schuyler A. Herres  
BY Thomas G. Miller  
FOR Green, McCallister & Miller  
HIS ATTORNEYS

June 2, 1953

S. A. HERRES

2,640,860

APPARATUS FOR MELTING TITANIUM TO FORM INGOTS

Filed Oct. 21, 1949

6 Sheets-Sheet 6



*Fig. 17*

INVENTOR.

Schuyler A. Herres

BY Thomas G. Miller

FOR Green, McCallister & Miller

HIS ATTORNEYS

## UNITED STATES PATENT OFFICE

2,640,860

APPARATUS FOR MELTING TITANIUM  
TO FORM INGOTSSchuyler A. Herres, Albany, N. Y., assignor to  
Allegheny Ludlum Steel Corporation, Bracken-  
ridge, Pa., a corporation of Pennsylvania

Application October 21, 1949, Serial No. 122,717

8 claims. (Cl. 13—9)

1

This invention pertains to improved procedure and apparatus for melting titanium metal and titanium base metal. One phase of my invention pertains particularly to the employment of a consumable electrode of titanium metal or titanium base alloy metal in an arc furnace or crucible.

In accordance with my invention, a consumable electrode is made by pre-forming titanium powder or titanium sponge metal up to one inch in particle size at a pressure of approximately 15 tons per sq. in. to form sticks of convenient length and cross section. The pressing is preferably carried out at room temperature and additions of other metals or compounds may be incorporated in the stick to provide alloy ingots of any desired composition. That is, the desired percentages of metal elements such as iron, chromium, molybdenum, tungsten, manganese, nickel and other alloying elements may be initially proportioned to the titanium powder or sponge metal and ground to suitable particle sizes up to one inch, mixed with the titanium powder or sponge metal, and then press-formed with the latter into the sticks. If gaseous elements such as oxygen and nitrogen are to be employed as alloying elements, relatively small proportions of oxides or nitrides of the alloying metals may be employed instead of the pure metals, provided that the electrical conductivity of the sticks is not appreciably affected. For this purpose, the core may be titanium metal with the metallic compounds as a surface layer thereabout.

The pre-formed sticks are continuously and progressively fed endwise as electrodes into an arc-melting furnace or crucible at a rate depending upon the rate of melting, to thereby build up an ingot. The rate of feed is preferably adjusted to provide an arc voltage of about 30 volts; the rate of melting is regulated within wide limits by the arc amperage. Either A. C. or D. C. may be used for the arc current. Although I have joined the preformed sticks together by mechanical fastenings, I prefer to secure them by an auxiliary flash welding circuit as they are being fed towards or into the furnace; threaded sticks, electric resistance welding, etc. may also be employed.

Also, in accordance with my invention, additional titanium metal, alloying elements (metals and gases) may be introduced directly into the furnace during the electrode melting operation and the metal elements melted along with a consumable titanium electrode or a plurality of electrodes, if used. An ambient atmosphere is maintained about the titanium-base sticks, as well as within the furnace and about a delivery end thereof that is non-contaminating of the titanium. Gases which are inert to titanium,

2

such as argon, helium and neon, or a vacuum may be employed for this purpose.

When the ingot has been built up to a sufficient depth or length, the arcing current may be turned off, the electrode feed stopped, the bottom of the furnace removed, the solidified ingot dropped, and the complete ingot removed or a major portion thereof severed from a portion retained in the furnace for again initiating the melting arc. I provide means for sawing off the ingot within an airlock chamber and for periodically delivering the sawed-off ingot through an airlock when it has cooled sufficiently to be non-reactive with atmospheric gases.

15 In the structural arrangements for illustrating the principles of my invention, Figure 1 is a top plan view of a melting and feed apparatus constructed in accordance with my invention;

20 Figure 2 is a side sectional view in elevation taken along the line II—II of Figure 1 and also showing additional apparatus for supplying welding current, arc current, and for removing ingots that have been formed;

25 Figure 3 is a side sectional view in elevation taken along the line III—III of Figure 1 and also showing fluid means for actuating a stick-feeding mechanism;

30 Figure 4 is a sectional detail of a portion of the feeding mechanism of Figure 3, showing it in an inoperative or raised position as compared to the operative or lowered position of Figure 3;

Figure 5 is a horizontal sectional view taken along the line V—V of Figure 3;

35 Figure 6 is a horizontal section taken along the line VI—VI of Figure 4;

Figure 7 is a horizontal section taken along the line VII—VII of Figure 2 and particularly illustrates details of a positive stick-feeding mechanism, as provided by a pair of driven rolls;

40 Figure 7A is a horizontal sectional view taken along the line VIIA—VIIA of Figure 2;

Figure 8 is a horizontal section taken along the line VIII—VIII of Figure 2 and illustrates a pair of idler rollers for guiding the sticks;

45 Figure 9 is a section similar to that of Figure 7, but illustrates a modified type of feeding mechanism for round sticks;

50 Figures 10 and 11 are vertical sectional views somewhat diagrammatically illustrating a method of forming the sticks;

Figure 12 is a vertical sectional detail in elevation through a lower portion of the structure of Figure 1, taken along the line XII—XII of Figure 13 and showing a lowered position of a bottom wall of the furnace as effected by a swing arm, prior to removing an ingot; in Figure 2, the furnace bottom wall is shown in a raised position incident to an arc-melting operation;

Figure 13 is a horizontal sectional view taken

through a top portion of an enclosure for the bottom of the furnace of Figure 2 and illustrating the operation of the furnace bottom wall swing arm of Figure 12 and of a swingable arm carrying an ingot-cutting saw mechanism:

Figure 14 is a vertical sectional view in elevation taken along the line XIV—XIV of Figure 13;

Figure 15 is a vertical sectional view showing details of the structure employed within the enclosure for the bottom of the furnace and taken along the line XV—XV of Figure 13:

Figure 16 is a horizontal sectional view taken along the line XVI—XVI of Figure 15 and showing ingot delivery structure; and,

Figure 17 is a somewhat diagrammatic view in elevation illustrating a circuit that may be employed for simultaneously operating three consumable electrodes in separate furnaces or in a common furnace; this view illustrates how three-phase A. C. current may be employed for supplying current to a plurality of electrodes.

Referring particularly to Figure 2 of the drawings, I have shown a crucible or furnace 10 provided with a jacketed cooling chamber A and defined by inner walls 11a, outer walls 11b, a top wall 12a and a bottom wall 12b. Cooling fluid, such as water, may be circulated through the chamber A by means of an inlet 11c and an outlet 11d. The inner wall 11a is preferably of copper, while the outer wall 11b may be of steel or a suitable alloy.

A top cover plate member 14 is securely mounted on the top wall 12a by means of bolt and nut assemblies 15. The cover plate member 14 is insulated from the top wall 12a by an insulating and fluid-sealing-off gasket 13 located therebetween and by insulating sleeves 13a about the bolt and nut assemblies 15.

A central melting chamber is defined by the inner or lining walls 11a and may be evacuated of contaminating gases through a passageway 14a in the cover member 14 and an outlet 14b. If, as also contemplated, the melting chamber is to be supplied with a non-contaminating gaseous atmosphere of a suitable gas such as argon, helium, or neon, a pair of passageways 14a and connections 14b may be provided, one for introducing the non-contaminating gas and the other for exhausting partially contaminated gas.

The top cover member 14 is also shown provided with an enclosure 17 about a center feed opening 16 therethrough that carries gasket material 18 to prevent the introduction of atmospheric gases into the furnace 10 to, if desired, seal off the furnace chamber from a superimposed feed enclosure 20—20'. An outwardly and upwardly sloped feed pipe 19 is shown extending through the top or cover plate member 14 and is provided with a threaded cap 19a and a gasket 19b for closing it off from the atmosphere. The pipe 19 may be used to introduce alloying metals or elements, or such elements with a non-contaminating gas.

Above the top of the melting furnace or crucible 10, I have shown the two-part feed chamber enclosure 20—20' which may be evacuated through a connection 20a or may be provided with a flow of non-contaminating gas by a pair of such connections. The bottom part 20' of the enclosure may be secured as by welding to the top plate member 14. The upper part 20 of the enclosure has a top closure wall 31 provided with a central feed opening therethrough; the latter is defined by a rectangular feed or

guide flange 32 (if the sticks are of rectangular cross-section) or by a circular or annular feed and guide flange 32 (if the sticks are of rounded section, see Figure 9). The flange 32 extends vertically into the feed chamber. It will be noted that the flange 32 at its top has a cone-shaped opening to permit easy introduction of a stick, such as B'' and terminates in a portion of uniform and lesser diameter (slight clearance is provided with the stick) which holds the stick in a vertically aligned relationship as it is fed therewith. Upper and lower roll pairs 21a—21b and 21'a—21'b are located in a vertically spaced-apart relationship within the chamber defined by the enclosure 20—20' to receive sticks and guide them into the crucible 10. The upper set, as shown in Figures 3 and 8, are idler rolls and the lower set, as shown in Figures 3 and 7, are positive feed rolls.

The upper part 20 of the enclosure has a bottom rim flange 20b and the lower part 20' has a top rim flange 20'b that abut on an electrical insulating and fluid sealing gasket 20c that is interposed therebetween. Insulating sleeves 20d extend through the flanges 20b, 20'b, and the gasket 20c and are adapted to receive nut and bolt assemblies 20e for securing the rim flanges together.

Referring particularly to Figures 3 and 7, the illustrated lower pair of rolls 21'a and 21'b have spaced-apart flanges 22 for guiding a stick of square or rectangular cross-section and shafts that are journaled at their opposite ends by bearings 23' and 24'. The bearings 23' and 24' are mounted on cross pieces or members 33' that are secured at their ends to the enclosure part 20'. Insulating material 33'a is interposed between the bearings and the pieces 33 to, like the motor gear 26, prevent current supplied by line 12a from being shorted. The feed roll 21'a has a spur gear 25a splined or secured thereon; the feed roll 21'b has a similar spur gear 25b secured or splined thereon. It will be noted that the spur gears 25a and 25b mesh with each other and are driven by a motor gear 26 (of Micarta or other suitable non-conducting or electrical insulating material) which meshes with one of the spur gears 25b and is keyed on a shaft 27 of a speed reduction unit 28. The unit 28 is actuated through a coupling or connection 29 by the drive shaft of a motor 30. It will thus be seen that the rolls 21'a and 21'b may be positively driven at relatively slow speed to continuously feed a consumable electrode to the furnace 10. In Figure 9, I have shown a slightly modified construction wherein the feed rolls 21'c and 21'd are of concave shape to feed a circular stick or electrode Bx.

As shown in Figure 3, the upper pair of rolls (idler) 21a and 21b are of similar design and mounting to the lower or feed rolls 21'a and 21'b, except that they are not provided with means for positively driving them. Their bearings 23 and 24 are mounted in a similar manner by means of insulating material 33a and cross pieces 33 on the upper enclosure part 20. The rolls 21'a and 21'b are connected through bearings 23 to electrical line 11a.

In figures 10 and 11 I have somewhat diagrammatically shown a press 5 having a removable bottom 6 and a plunger 7 for compacting sponge or powdered titanium 8, etc. into a stick B.

In Figures 1, 2 and 3 to 6, inclusive, I have shown a carrier wheel or magazine 38 provided

with radially-extending spaced-apart compartments 38a for carrying individual electrode sticks, and means for feeding the sticks from a compartment that is in alignment with the feed flange 32 of the enclosure part 20. The compartments 38a preferably have a shape corresponding to the shape of the sticks to be carried therein. In accordance with my invention, the electrode sticks which may be of any suitable cross section, but are preferably rectangular, are press-formed (see Figures 10 and 11), delivered to the compartments 38a of the carrier 38 (see Figure 5) through an airlock delivery chute 65 (see Figure 3), and are then intermittently pushed through the feed flange 32.

I have provided an enclosure 35 that is superimposed on the feed enclosure part 20 and that encloses the carrier wheel 38 which is adapted to be rotated intermittently. The carrier wheel 38 is splined or secured on a central, vertical shaft 39 which at its lower end is journaled within bearings 41a mounted in an offset or depressed portion 37a of the top wall 31 of the feed enclosure part 20. At its other end, the shaft 39 is journaled within a bearing 41b which is carried by a bearing box 40 mounted on a top wall 37 of the enclosure 35. It will be noted that the cylindrical side wall or shell 36 of the enclosure 35 extends in a spaced-apart relationship about the rotatable carrier feed wheel or casting 38 and is secured on the top wall 31 of the feed enclosure part 20 by bolt and nut assemblies 34.

As shown particularly in Figures 1, 2 and 5, a sprocket wheel 42 is keyed on a top end of the shaft 39 and is driven by a chain 43 and a sprocket wheel 44. The sprocket wheel 44 is splined or secured to a drive shaft 45 of an actuating motor 46. The motor 46 is provided with a slip coupling 45a between two parts of its shaft 45, so that the wheel 38 will rotate until one of the sticks in one of its compartments 38a aligns with the feed flange 32 and falls or is moved through a feed hole in the bottom of the enclosure 35 to stop the rotation of the wheel. At such time, the coupling 45a slips and permits the motor 46 to continue to rotate. Such stick is then forced downwardly between the upper pair of feed rolls 21a and 21b by a piston pusher head 49b. The rotation of the wheel 38 is not resumed until the stick has been fully fed out of its compartment 38a and the piston pusher head 49b has been drawn upwardly out of the compartment into an offset portion 37a of the top wall 37. At this time, the wheel 38 is again slowly rotated to position the next compartment 38a in an endwise aligned feeding position with the feed flange 32, and the operation continued.

As shown in Figures 2, 3, 5 and 6, a slide plate member 60 is operably positioned between a slotted top face 31b of the wall 31 of enclosure part 20 and a bottom edge of the side wall 36 of the enclosure 35. The member 60 is thus adapted to slide along the slot 31b in the wall 31 to cover its feed opening; it is used to prevent any sticks from dropping endwise into the feed flange 32 when the compartments of the carrier wheel 38 are being preliminarily filled with sticks. A flange 62 is secured to the wall 36 to extend fully around the slot 31b and a depression or offset 31c in the top face of the wall 31 carries gasket material 63 for sealing off the slide joint provided with the member 60. As shown in Figures 5 and 6, the slide member 60 has an operating handle 61. An offset abutment portion 60a cooperates with a pin 31d that ex-

tends upwardly from the wall 31 to limit the maximum outward movement of the slide member 60.

The wheel of Figure 5 will receive eight sticks; 5 the selected number of compartments 38a will depend on the desired size of ingot to be built up in the furnace 10. That is, I contemplate refilling the carrier wheel 38 while a formed ingot is being dropped and severed at the bottom of

10 the furnace.

Referring particularly to Figures 2, 3, 4, 5 and 6, a piston cylinder or chamber wall 50 of a fluid motor is secured as by bolts 48 to the top wall 37 of the enclosure 35 and carries a piston head 49a that is mounted on an upper end of a piston rod 49. The pusher head 49b is mounted on the lower end of the rod 49. It will be noted that the piston head 49a is adapted to slide up and down within the chamber defined by the cylinder wall 50 and that the pusher head 49b is adapted to slide up and down within a periodically aligned compartment 38a. The head 49b is adapted to be withdrawn or raised out of the compartment 38a into the offset portion 37a in the top wall 37 of the enclosure 35. A top wall 51 is secured over the cylinder 50 and carries a pressure relief and safety valve 52a; a second valve 52b of the same type is mounted in the lower end of the cylinder 50.

15 20 25 30 35 40 45 50 55 60 65 70 75

The cylinder 50 is provided with a passageway 51a into its upper end and a passageway 51b into its lower end for supplying hydraulic or any suitable pressure fluid to opposite ends of the piston 49a to move it up and down within the chamber of the cylinder. The passageway 51a is connected to line 53 and the passageway 51b is connected to line 54. A dual-acting control valve 55 is spring-actuated to shut off flow through both the lines 53 and 54 when the piston 49a is in its upper position and the slide plate 60 has moved to its inner position. When the slide plate 60 is moved to its outer position, it presses an operating arm 56 of the valve 55 to an open position against the tension of its spring, thus permitting fluid to flow along both of the lines 53 and 54. Packing 50a is positioned within the lower end of the cylinder 50 and about the rod 49 to seal off the piston chamber.

A double-acting line-reversing valve 57 is positioned in the fluid lines 53 and 54 beyond the valve 55. The valve 57 is actuated by an arm 58 to either cause a positive flow through line 53 by connecting it to supply line 53a and a return flow through line 54 by connecting it to return line 54a, or to cause a positive flow through line 54 by connecting it to supply line 53a and a return flow through line 53 by connecting it to the return line 54a. By reversing the valve 57, the piston 49a can be moved up and down within its cylinder 50 to push an endwise-aligned stick out through the feed flange 32, withdraw the pusher 49b, permit the carrier 38 to rotate one step and present the next successive stick, and then push it endwise through the feed flange 32 and between the upper pair of guide rolls 21a and 21b.

The carrier 38 is slowly rotated while the sticks are fed into the compartments 38a through a chute 65 (see Figure 3). The chute 65 extends upwardly from the top wall 37 of the enclosure 35 and is normally closed by a cover lid 66 that is hinged at 67 and locked in position by a thumb-nut and pivot pin assembly 69. The assembly 69 is pivoted at 70 to the chute and is adapted to extend into an open-end slot 66a of the lid 66. A gasket 68 seals off the cover 66 when it is in

its closed position. During the filling of the compartments **38a**, the pusher **49b** is raised to its extreme upper position to clear the carrier **38**, the closure plate **60** is moved inwardly to close up the opening in the bottom of the chamber of the enclosure **35**, the valve **55** is shut off, and the carrier **38** is rotated by the motor **46** to progressively present each of the compartment openings **38a** to the feed chute.

Referring to Figure 2 of the drawings, the bottom of the furnace **10** is closed off by a bottom plate or wall **76** that is carried by a swing arm member **75** and is secured as by brazing within the wall portions of an opening **75a** therethrough. The opening **75a** corresponds in diameter to the inner diameter of the wall **11a** of the furnace **10** that is closed off at its top by the bottom plate **76** (preferably of copper). A plate **77** (preferably of ferrous metal) is secured as by welding on a bottom face of the member **75** to close off the bottom of the opening **75a** and to, with the plate **76**, define a cooling chamber **D** through which cooling fluid such as water is circulated by inlet and outlet connections **77a** and **77b**.

In Figure 2 I have indicated starting metal in the furnace **10** by **C**, a small portion of which may be inserted therein to start the operation and which will then build up as the electrode sticks **B**, **B'**, **B''**, etc. are melted down. After an ingot **I** of suitable size has been built up, the arm member **75** may be lowered and swung out of position and the ingot removed or cut off, as shown in Figures 14 and 15, within a bottom, sealed-off enclosure **90**. The enclosure **90** has a connection **90a** that may be employed to apply a vacuum, or may have a pair of such connections for supplying and exhausting an inert gas.

The construction of the swingable arm member **75** which carries the bottom wall **76** of the crucible or furnace, is shown particularly in Figures 2, 12 and 13. It will be noted that it is positioned vertically by a pair of fluid-actuated motors **88** that are secured to extend upwardly from floor stands **81** and are actuated by inlet and outlet connections **88a** and **88b** to raise and lower their pistons **89** and to thus raise and lower the member **75** on a vertical pivot pin **79**. A threaded-on nut **79a** serves as a stop to limit the maximum extent of the upward movement of arm member **75** on the pin **79**. A bearing sleeve **80a** extends through the arm member **75** and about the pin **79**.

A swing pin **82** extends upwardly through a bearing sleeve **89b** in an end of the arm **75** and is reduced and threaded at its lower end for mounting on a piston rod **83** of a fluid-actuated motor **84**. A nut **82a** secures a reduced and threaded end of the pin **82** on the rod **83**. It will be noted that the arm member **75** is free to move vertically up and down on the pins **79** and **82** when the fluid motors **88** are operated. In this manner, the bottom wall **76** of the furnace can be raised and lowered out of position with respect to the inner wall **11a** thereof. The motor **84** which operates to swing the arm **75** is actuated by fluid connections **84a** and **84b** and its integral end portion **85** is mounted on a standard **87** by a pin or bolt **86** which extends through a bifurcated portion of the standard **87**. As shown particularly in Figure 13, the arm member **75** can be swung from a normal position **E** in alignment with the bottom of the furnace **10** to a side position **F** when an ingot is to be removed or sawed off.

Referring particularly to Figures 13, 14, 15 and 16, I have shown a saw mechanism which like

the arm member **75** and its associated mechanism is mounted within the enclosure **90**. The saw mechanism has a rotating saw blade **107** provided with a shaft **108** splined thereto (see Figure 14). The shaft **108** is journaled on a swing arm **111** and carries a sprocket wheel **109** which is secured on its lower, reduced, threaded end **108a** by a mounting nut **110**. A chain **116** meshes with the sprocket **109** and is driven by a sprocket **115** that is splined or secured on an actuating shaft **112**. The shaft **112** also has a second sprocket wheel **117** secured thereto and driven by a chain **118** and a sprocket **119** of a gear reduction unit **120**. The shaft of an electric motor **121** is coupled to the unit **120**. The shaft **112** is journaled at its lower end in a mounting **113** and at its upper end **112a** is reduced, threaded, and journaled within the swing arm **111**. A nut and washer assembly **114** holds the swing arm **111** pivotally in position on the reduced end **112a** of the drive shaft **112**.

An opposite end of the arm **111** is actuated by a swing link pin **122** which extends through a bifurcated end **124a** of a piston rod **124** which is actuated by a fluid motor **125**. Actuating fluid is introduced and exhausted from the motor **125** by connections **125a** and **125b**. The motor **125** has an integral extension **126** that is secured within the bifurcated portion of a standard **128** by a pin or bolt **127**. As shown particularly in Figure 13, the arm **111** and its associated saw **107** is adapted to be moved from an inoperative position **G** to a sawing position **H** when the bottom wall **76** of the furnace or crucible has been lowered by the arm member **75** and swung to outer position **F** of Figure 13. The fluid motors **84** and **125** are of a double-acting type, so that they can be moved positively in either direction. The motors **88** may be of either a single- or double-acting type.

To support the build-up ingot **I** when the bottom **76** of the furnace has been removed, see Figures 14 and 15, I have provided a fluid motor **104** which has a piston rod **105** and a support head **105a** that is adapted to move through an opening **100a** in a delivery chute **100**. Fluid is supplied to and exhausted from the motor **104** by connections **104a** and **104b** and it is preferably double-acting. As shown in Figure 14, the motor **104** supports the bottom of the ingot **I**, after its weight moves it out of the furnace **10** and into a sawing position. The length of ingot which is cut can thus be governed by the vertical position of the head **105a** of the motor **104**. As shown in Figure 15, the major portion or length **I'** of the ingot is supported by the vertically movable head or table **105a** during the sawing-off operation. The remainder of the ingot **I** is of relatively short length and thus of relatively slight weight and is free to move vertically-upwardly within the guiding walls of the crucible or furnace **10**. The table **105a** is preferably lowered slightly during the operation to ease off the lower ingot portion **I'**. Thus, no difficulty is encountered from the standpoint of a binding of the saw during the cutting-off operation.

After an ingot **I** has been sawed off, as shown particularly in Figures 15 and 16, the head **105a** can be lowered, as shown by the dot and dash lines of Figure 15, and the cut-off ingot **I'** will fall into the delivery chute **100** and move to the full line position shown, to the right of this figure.

The inclined chute **100** is mounted on a standard **103** at its upper end and on a standard **101** at its lower end. As shown particularly in Figure 16, it is provided with side walls **100b**, an upper

end wall 100c, and an abutment end wall 102 for guiding and positioning the cut-off ingot I'.

A supplemental airlock chamber is provided at the delivery end of the enclosure 90 and is defined by an enclosure 91, see Figures 15 and 16. An opening 90a through a vertical wall of the enclosure 90 permits ingots to be delivered to the airlock chamber of the enclosure 91. It will be noted that the inclined chute 100 also rests upon a lower portion of the wall 90b of the enclosure 90. A door 96 having a handle 96a is slidably mounted on the wall of the enclosure 90 by flanges 97 and sealing-off gasket material 98 to normally close off the opening 90a. The door 96 is raised when an ingot I' is to be delivered and is then moved down against the chute 100. The top wall of the airlock enclosure 91 has an opening 91a therein for lifting out an ingot from the lower end of the chute 100. A horizontally-slidable door 92 normally seals off the opening 91a. The door 92, as shown in Figures 15 and 16, has a handle 92 and is mounted in flanges 93 and 97 and sealed off by gasket material 94 and 98.

Referring particularly to Figure 2 of the drawings, I have shown a pair of motor-generator sets 70a and 70b that are connected in parallel for supplying D. C. current for welding adjacent sticks, such as B' and B'' together. The set 70b also provides arcing current for the furnace 10. The motor generator set 70a on its positive side is connected through a line 71a, switch 73a, and bearings 23 (see Figure 8) to the upper pair of rolls 21a-21b. Its negative side is connected by a line 72a to the negative side 72b of the other set 70b and through bearings 23' (see Figure 7) to the lower pair of feed rollers 21'a-21'b. The positive side of the motor generator set 70b is connected by a line 71b, switch 73b, and a flexible cable 71'b' to the arm 15, and thus, to the furnace bottom 76. It will thus be apparent that when the switch 73b is closed, arcing current of one potential will be supplied to the unitary electrode B'-B'' and arcing current of opposite potential will be supplied to the metal C through the furnace bottom 76. Thus an arc will be established between C and B of Figure 2.

When an upper electrode stick, such as B'' is to be secured (as by flash-welding) to a lower stick such as B', it is fed into an endwise abutting relationship with the lower stick (see Figure 3) by the pusher 49a, is aligned in such position by the idler guide rolls 21a-21b, and current of one potential is then supplied through the line 71a to the stick B'' by closing the switch 73a. Current of opposite potential is applied to the other stick B' through line 72a. After the welding operation, the switch 73a is opened.

The pusher 49a keeps the stick B'' in welding abutment with the stick B' during the welding operation, although the latter is being advanced slowly into the furnace 10 by the driven feed rolls 21'a and 21'b. After the welding operation, the pusher 49a may be raised and the welded sticks will then be fed as unitary electrode by the rolls 21'a and 21'b.

In Figure 17 I have disclosed a utilization of three-phase alternating current for supplying energy to a plurality of consumable electrodes. In this diagram P<sub>1</sub>, P<sub>2</sub> and P<sub>3</sub> are primaries for the various phases of an A. C. transformer, while S<sub>1</sub>, S<sub>2</sub> and S<sub>3</sub> are corresponding secondaries thereof. Switches S and individual phase transformers having primary taps T and primaries and secondaries P<sub>4</sub>-S<sub>4</sub>, P<sub>5</sub>-S<sub>5</sub> and P<sub>6</sub>-S<sub>6</sub>, respectively,

are shown. The secondaries S<sub>4</sub>, S<sub>5</sub> and S<sub>6</sub> are connected through switches S<sub>w</sub> to the upper roll pairs 21a and 21b for effecting a welding operation between adjacent electrode sticks. Switches S<sub>w</sub> are located in one lead from each phase secondary to turn off the arc-producing current for each electrode when desired. The other lead of each phase secondary is connected to the lower set of feed rolls 21'a-21'b. Although I have shown a plurality of furnaces or crucibles 10 actuated by the three-phase A. C. circuit, it will be apparent that a single furnace or crucible may be used and provided with a plurality of feed openings for feeding a plurality of sticks, if a larger size of ingot is to be produced. As shown, the number of transformers used will depend upon the number of phases of the A. C. current source.

Although it has been customary to employ a direct current source of energy where a non-consumable electrode is used and to connect its negative lead to the electrode to minimize its deterioration, alternating current has been found to be suitable where the electrode is of a consumable type. As shown in Figure 2, I prefer to connect the positive lead of a direct current source to a consumable electrode to increase its melting rate.

What I claim is:

1. In apparatus of the character described for making metal ingots in a furnace crucible utilizing a consumable electrode made up of pre-formed sticks of air-sensitive metal, the combination of a carrier provided with a series of stick-receiving compartments therein, a sealing-off enclosure for said carrier, a second sealing-off enclosure positioned beneath said first-mentioned enclosure and on the furnace crucible over an opening therein, an opening through the top of said second enclosure into said first enclosure, guide means positioned within said second enclosure in alignment with the top opening therein and having portions to guide sticks through the opening of and into the furnace crucible, means actuating said carrier to periodically and progressively align each of its compartments with the top opening in said second enclosure, and means operably positioned within said first enclosure to advance a stick from an aligned compartment of said carrier through the top opening of said second enclosure into engagement with said guide means.

2. In an apparatus as defined in claim 1 wherein, said last-mentioned means is a pusher operably positioned for movement along an aligned compartment of said carrier and operably connected to a fluid motor.

3. In an apparatus as defined in claim 2 wherein, said guide means has a pair of pass-defining, positively-driven feed rolls; said pusher is adapted to be periodically actuated by said fluid motor at a faster rate than the rate of feed of said feed rolls to move a second stick from a second aligned compartment of said carrier into endwise abutment with the first-mentioned stick that is within the pass of said pair of feed rolls, and means positioned within said second enclosure to weld the abutting sticks together into a unitary electrode.

4. In apparatus of the character described for making metal ingots in a furnace crucible utilizing a consumable electrode made up of pre-formed sticks of an air-sensitive metal, the combination of a carrier provided with a series of stick-receiving compartments therein, a sealing-off en-

## 11

closure for said carrier, a second sealing-off enclosure positioned beneath said first-mentioned enclosure and on the furnace crucible over an opening therein, an opening through the top of said second enclosure into said first enclosure, means actuating said carrier to periodically and progressively align each of its compartments with the top opening of said second enclosure, means operably positioned within said first enclosure to advance a stick endwise from an aligned compartment of said carrier through the top opening thereof into said second enclosure, guide means operably positioned in said second enclosure to receive successive sticks from periodically aligned compartments of said carrier and advance them into the furnace crucible, and electric welding means operably associated with said guide means and positioned in said second enclosure in alignment with the path of movement of the sticks therethrough and having portions connected to welding current of opposite potential to weld abutting edges of a pair of sticks together into a unitary electrode before they are introduced into the furnace crucible.

5. In apparatus of the character described for making metal ingots in a furnace crucible utilizing a consumable electrode made up of pre-formed metal sticks, the combination of a carrier provided with a series of stick-receiving compartments therein, a sealing-off enclosure for said carrier, a second sealing-off enclosure positioned beneath said first-mentioned enclosure and on the furnace crucible over an opening therein, an opening through the top of said second enclosure into said first enclosure, means actuating said carrier to periodically and progressively align each of its compartments with the top opening of said second enclosure, means operably positioned within said first enclosure to advance a stick endwise from an aligned compartment of said carrier through the top opening thereof into said second enclosure, guide means operably positioned in said second enclosure to receive successive sticks from periodically aligned compartments of said carrier and advance them into the furnace crucible, said guide means comprise an upper pair of rolls in operative engagement with one of the sticks to be welded, and a lower pair of rolls in operative contact with the other of the sticks to be welded; a source of current of one potential adapted to be connected to intermittently supply said upper pair of rolls, a source of current of opposite potential continuously connected to supply said lower pair of rolls, means connecting the source of current of one potential to the furnace crucible, and the current of opposite potential connected to said lower pair of rolls being supplied by its source to the electrode provided by the welded sticks for effecting the arc melting operation within the furnace crucible.

6. In an apparatus as defined in claim 5 wherein, means is provided for actuating said lower pair of rolls to advance the welded electrode into the furnace crucible, and said means for advancing a stick from an aligned compartment of said carrier has means for reciprocating it to advance a stick therein into abutment with a preceding stick that is being advanced by said lower pair of rolls and to withdraw and advance another stick into abutment with the second stick.

7. In an arc melting furnace apparatus of the character described for making ingots from pre-formed composite consumable electrode sticks of

## 12

an air-sensitive metal, the combination of a rotatable carrier wheel provided with a series of radially-positioned stick-receiving compartments, an enclosure about said wheel, means rotatably mounting said wheel within said enclosure, a feed chute mounted on said enclosure for feeding sticks into the compartments of said wheel as it is rotated, said feed chute having an air-lock for normally excluding contaminating gases from said enclosure, a pusher means operably mounted on said enclosure above the path of movement of the compartments of said wheel, a feed opening through the bottom of said enclosure, means for periodically moving said pusher means into and along each of the compartments of said wheel to push a stick out through the opening in the bottom of said enclosure, a second enclosure about the bottom of said first-mentioned enclosure and having a feed portion open to and in alignment with the feed opening in said first-mentioned enclosure, vertically spaced-apart pairs of rolls operably mounted in said second enclosure in an aligned-stick-feeding relationship with respect to each other, said pusher means having a path of operative movement sufficient to push a stick from each compartment of said wheel into a pass formed by an upper pair of said rolls, a lower pair of said rolls having a spaced relationship with respect to said upper pair that is shorter than the length of a stick being fed, said second-mentioned enclosure being mounted on the arc-melting furnace and having an opening through a bottom thereof into the furnace, and means for actuating said lower pair of rolls to advance a stick through the opening in the bottom of said second enclosure into the furnace to provide an electrode therefor.

8. In an apparatus as defined in claim 7 wherein, said upper pair of rolls is positioned to guide a second stick into abutment with a stick within in the pass of said lower pair of rolls, and means is provided for supplying electric current of opposite potential to said upper and lower feed roll pairs to weld the abutting sticks together to form a unitary electrode for the furnace.

SCHUYLER A. HERRES.

References Cited in the file of this patent

UNITED STATES PATENTS

| Number       | Name             | Date          |
|--------------|------------------|---------------|
| 559,731      | McDonald         | May 5, 1896   |
| 623,075      | Chamberlain      | Apr. 11, 1899 |
| 1,491,964    | Moxham           | Apr. 29, 1924 |
| 55 1,807,090 | Pistor           | May 26, 1931  |
| 2,019,727    | Quinn et al.     | Nov. 5, 1935  |
| 2,060,074    | Heuer            | Nov. 10, 1936 |
| 2,117,913    | Seil             | May 17, 1938  |
| 2,121,280    | Bell             | June 21, 1938 |
| 2,140,607    | Thompson         | Dec. 20, 1938 |
| 2,143,987    | Koller           | Jan. 17, 1939 |
| 2,148,391    | McBride          | Feb. 21, 1939 |
| 2,163,967    | Strawn et al.    | June 27, 1939 |
| 2,205,854    | Kroll            | June 25, 1940 |
| 65 2,264,287 | Betterton et al. | Dec. 2, 1941  |
| 2,356,338    | Misfeldt         | Aug. 22, 1944 |
| 2,433,032    | Dempsey et al.   | Dec. 23, 1947 |
| 2,445,670    | Hopkins          | July 20, 1948 |
| 2,477,258    | MacMillin        | July 26, 1949 |
| 2,541,764    | Herres et al.    | Feb. 13, 1951 |

OTHER REFERENCES

Project Rand, Titanium and Titanium-Base Alloys, Battelle Memorial Institute, Columbus, Ohio, Mar. 15, 1949, pp. 56, 57, and 58.